



US009670738B2

(12) **United States Patent**  
**Overstreet**

(10) **Patent No.:** **US 9,670,738 B2**  
(b4) **Date of Patent:** **Jun. 6, 2017**

(54) **METHODS OF FORMING A HARDFACING COMPOSITION, METHODS OF HARDFACING A DOWNHOLE TOOL, AND METHODS OF FORMING AN EARTH-BORING BIT**

(71) Applicant: **Baker Hughes Incorporated**, Houston, TX (US)

(72) Inventor: **James L. Overstreet**, Tomball, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 765 days.

(21) Appl. No.: **13/953,351**

(22) Filed: **Jul. 29, 2013**

(65) **Prior Publication Data**

US 2013/0305617 A1 Nov. 21, 2013

**Related U.S. Application Data**

(63) Continuation of application No. 12/893,953, filed on Sep. 29, 2010, now Pat. No. 8,540,036.

(60) Provisional application No. 61/246,711, filed on Sep. 29, 2009.

(51) **Int. Cl.**

*C22C 29/08* (2006.01)  
*E21B 10/46* (2006.01)  
*B24D 99/00* (2010.01)

(52) **U.S. Cl.**

CPC ..... *E21B 10/46* (2013.01); *B24D 99/005* (2013.01)

(58) **Field of Classification Search**

None

See application file for complete search history.

(56) **References Cited**

**U.S. PATENT DOCUMENTS**

|                   |        |                                       |                                             |
|-------------------|--------|---------------------------------------|---------------------------------------------|
| 4,196,233 A       | 4/1980 | Bitzer et al.                         |                                             |
| 6,124,564 A *     | 9/2000 | Sue ..... B23K 9/287<br>175/327       |                                             |
| 7,666,244 B2      | 2/2010 | Lockwoodl<br>2002/0017507 A1 *        | 2/2002 North ..... B23K 9/048<br>219/121.45 |
| 2003/0000339 A1 * | 1/2003 | Findeisen ..... B22F 1/0048<br>75/240 |                                             |
| 2003/0079565 A1   | 5/2003 | Liang et al.                          |                                             |
| 2006/0005662 A1 * | 1/2006 | Lockwood ..... E21B 10/50<br>75/240   |                                             |
| 2007/0090168 A1 * | 4/2007 | Snow ..... B23K 9/28<br>228/101       |                                             |

(Continued)

**FOREIGN PATENT DOCUMENTS**

GB 499789 \* 7/1937

*Primary Examiner* — Jessee Roe

*Assistant Examiner* — Ngoclan T Mai

(74) *Attorney, Agent, or Firm* — TraskBritt

(57) **ABSTRACT**

A hardfacing composition for downhole well tools, such as earth-boring bits, contains sintered ultrahard particles. The ultrahard particles consist of tungsten carbide grains, cobalt and vanadium. The ultrahard particles are dispersed within a matrix metal of iron, nickel or alloys thereof. The composition may also have sintered tungsten carbide particles of a larger size than the ultrahard particles. The ultrahard particles have a greater hardness than the sintered tungsten carbide particles. The ultrahard particles and the sintered tungsten carbide particles may be in a spherical pellet form. Other hard metal particles may be in the composition.

**14 Claims, 5 Drawing Sheets**



(56)

**References Cited**

U.S. PATENT DOCUMENTS

- 2008/0302702 A1\* 12/2008 Devakottai ..... C10G 9/16  
208/132  
2008/0311306 A1\* 12/2008 Xiao ..... C04B 35/478  
427/453  
2010/0113250 A1\* 5/2010 Tsunoda ..... C22C 1/051  
501/94  
2010/0230173 A1\* 9/2010 Xia ..... E21B 10/50  
175/374  
2011/0000715 A1\* 1/2011 Lyons ..... B23K 35/36  
175/374  
2011/0073378 A1 3/2011 Overstreet

\* cited by examiner

Fig. 1





Fig. 2  
(Prior Art)



Fig. 3



Fig. 4



Fig. 5



Fig. 6



Fig. 7



Fig. 8

## 1

**METHODS OF FORMING A HARDFACING COMPOSITION, METHODS OF HARDFACING A DOWNHOLE TOOL, AND METHODS OF FORMING AN EARTH-BORING BIT**

**CROSS-REFERENCE TO RELATED APPLICATIONS**

This application is a continuation of U.S. patent application Ser. No. 12/893,953, filed Sep. 29, 2010, now U.S. Pat. No. 8,540,036, issued Sep. 24, 2013, which claims the benefit of U.S. Provisional Patent Application Ser. No. 61/246,711, filed Sep. 29, 2009, the disclosure of each of which is hereby incorporated herein in its entirety by this reference.

**FIELD OF THE INVENTION**

This invention relates in general to hardfacing on earth-boring bits and, in particular, to a hardfacing containing a mixture of ultrahard sintered tungsten carbide pellets with other types of tungsten carbide pellets.

**BACKGROUND**

Hardfacing has been used for many years on earth-boring bits to reduce the abrasive and/or erosive wear. The hardfacing typically comprises hard metal particles dispersed within a metal matrix. The hard metal particles are often formed of tungsten carbide. Sintered tungsten carbide, also called cemented carbide, comprises tungsten carbide grains within a binder powder, such as cobalt. The tungsten carbide grains utilized in sintered tungsten carbide pellets are generally less than ten microns in diameter. During this sintering process, which employs heat and pressure, the cobalt will enter a liquid stage while the tungsten carbide grains remain in the solid stage. As a result of this process, the cobalt cements the tungsten carbide grains to create sintered tungsten carbide. The ductile cobalt metal offsets the characteristic brittleness of the tungsten carbide particles, resulting in a pellet that has enhanced toughness and durability. Sintered tungsten carbide pellets can be formed into generally spherical shapes or irregular shapes. Also, sintered tungsten carbide in a crushed form is available.

Cast tungsten carbide particles are formed in a casting process, and, thus, are harder than sintered tungsten carbide and do not have a binder of a soft metal such as cobalt. Cast tungsten carbide particles may be spherical, irregular or crushed. Spherical cast carbide pellets are typically smaller in diameter than standard spherical sintered tungsten carbide pellets. Cast tungsten carbide particles are thus harder than sintered tungsten carbide particles but more brittle.

Prior art hardfacing for earth-boring bits contains a variety of sizes and volume fractions of standard spherical sintered tungsten carbide pellets, crushed sintered tungsten carbide particles, spherical cast tungsten carbide pellets, crushed cast tungsten carbide particles, as well as other types of cast tungsten carbide, such as monocrystalline or macro-crystalline particles. The matrix that contains and binds the hardfacing pellets and particles is often iron, but it also may contain nickel and/or other alloys.

**SUMMARY**

The hardfacing composition described herein includes particles referred to herein for convenience as "ultrahard"

## 2

particles. The ultrahard particles are sintered and consist of tungsten carbide grains, cobalt and vanadium. The ultrahard particles are dispersed within a matrix metal of iron, nickel or alloys thereof. In one embodiment, the ultrahard particles comprise 4% to 8% cobalt, 0.25% to 2% vanadium, with the remainder being tungsten carbide.

The composition may also contain conventional sintered tungsten carbide particles, typically of a larger size than the ultrahard particles. The ultrahard particles have a greater hardness than the sintered tungsten carbide particles. The composition may also include cast tungsten carbide particles. The ultrahard particles have a lesser hardness than cast tungsten carbide particles but greater toughness. The ultrahard particles may be in a spherical form or a crushed form.

**BRIEF DISCUSSION OF THE DRAWINGS**

FIG. 1 is a side elevational view of an earth-boring bit having hardfacing in accordance with this invention.

FIG. 2 is a schematic photomicrograph illustrating a prior art hardfacing having sintered tungsten carbide pellets and spherical cast tungsten carbide pellets.

FIG. 3 is a schematic photomicrograph illustrating a hardfacing having ultrahard spherical sintered tungsten carbide pellets mixed with standard spherical sintered tungsten carbide pellets.

FIG. 4 is a schematic photomicrograph illustrating a hardfacing having ultrahard spherical sintered tungsten carbide pellets mixed with standard spherical sintered and cast tungsten carbide pellets.

FIG. 5 is a schematic photomicrograph illustrating a hardfacing having ultrahard and standard spherical sintered pellets mixed with ultrahard crushed sintered tungsten carbide particles.

FIG. 6 is a schematic photomicrograph illustrating a hardfacing having ultrahard and standard spherical sintered tungsten carbide pellets mixed with crushed cast tungsten particles.

FIG. 7 is a schematic photomicrograph illustrating a hardfacing having ultrahard and standard spherical sintered tungsten carbide pellets in combination with monocrystalline carbide particles.

FIG. 8 is a schematic photograph illustrating a hardfacing having ultrahard and standard spherical sintered tungsten carbide pellets with ultrahard crushed sintered tungsten carbide pellets, crushed cast tungsten carbide particles, and monocrystalline tungsten carbide particles.

**DETAILED DESCRIPTION OF THE INVENTION**

FIG. 1 illustrates an earth-boring bit 11 having a body 13. A threaded stem 15 extends upward from body 13 for connection to a string of drill pipe. Body 13 has at least one bit leg 17, typically three. A cone 19 is rotatably mounted to each bit leg 17. A lubricant reservoir supplies grease to the bearing spaces between each cone 19 and bit leg 17. A pressure compensator cap 21 encloses the upper end of each reservoir. Typically, each cone 19 is secured by retaining balls (not shown). The retaining balls are fed through a hole in each bit leg 17, and then the hole is plugged by a ball plug 23, which is welded to bit leg 17. After assembling a cone 19 on each bit leg 17, the three separate portions of body 13 are welded together. The fixture for holding the three portions in place during welding may engage a dimple 25 on the outside surface of each bit leg 17.

Bit 11 contains hardfacing in various places to prevent wear on the steel components. In this embodiment, bit leg outer surface hardfacing 27 covers the entire outer surface of each bit leg 17 except for ball plug 23 and fixture dimple 25. Hardfacing 27 extends from the lower end, or shirtpail, of each bit leg 17 to the recess containing pressure compensator cap 21. A leading edge hardfacing 29 extends over the leading edge of each bit leg 17. A trailing edge hardfacing 31 extends over the trailing edge of each bit leg 17. Leading edge hardfacing 29 and trailing edge hardfacing 31 join outer surface hardfacing 27.

A robotic process may serve as the method of applying hardfacing layers 27, 29 and 31. In a plasma transferred arc (PTA) process, hardfacing powder flows down a nozzle to an arc. The arc moves relative to the bit leg 17 during the application. Other methods are available, such as using an oxyacetylene torch and a rod. Some earth-boring bits 11 may have outer surface hardfacing 27 applied only on the lower edge or shirtpail. Some bits may have only leading edge hardfacing 29 and not trailing edge hardfacing 31. The compositions of outer surface hardfacing 27, leading edge hardfacing 29 and trailing edge hardfacing 31 may be the same or may differ.

Cones 19 also contain layers of hardfacing, particularly if it is a milled tooth type. In a milled tooth bit, cones 19 have rows of machined or milled teeth 33 that are formed integrally with the body of each cone 19. Teeth 33 contain layers of teeth hardfacing 35. Teeth hardfacing 35 covers the leading and trailing flanks and the inner and outer sides of each tooth 33. Each cone 19 has a gage surface that may contain a layer of gage hardfacing 37 for engaging the side wall of the bore hole. Teeth hardfacing 35 and gage surface hardfacing 37 are typically applied by heating with an oxyacetylene torch a metal tube filled with hard metal particles. The hardfacing layers 35, 37 on cones 19 often have different compositions than hardfacing layers 27, 29 and 31 on bit leg 17.

FIG. 2 illustrates a prior art example of the composition of hardfacing applied as one or all of the layers 27, 29, 31, 35 and 37. FIG. 2 illustrates standard spherical sintered tungsten carbide pellets 39 and spherical cast tungsten carbide pellets 41. Standard spherical sintered tungsten carbide pellets 39 are normally larger in diameter than spherical cast tungsten carbide pellets 41. Standard spherical sintered tungsten carbide pellets 39 have a binder, normally cobalt, which binds the carbide powder. Standard spherical sintered tungsten carbide pellets 39 are available in a variety of sizes from about 16 mesh on the larger size to about 325 mesh on the smaller size. Stated in another manner, the size range could be from about 45 micrometers ("microns") to about 1190 microns.

Sintered tungsten carbide, also called cemented carbide, comprises tungsten carbide grains within a binder powder, such as cobalt. The tungsten carbide grains utilized in standard spherical sintered tungsten carbide pellets 39 are generally less than ten microns in diameter. During this sintering process, which employs heat and pressure, the cobalt will enter a liquid stage while the tungsten carbide grains remain in the solid stage. As a result of this process, the cobalt cements the tungsten carbide grains to create sintered tungsten carbide. The ductile cobalt metal offsets the characteristic brittleness of the tungsten carbide particles, resulting in a pellet that has enhanced toughness and durability. Sintered tungsten carbide pellets can be formed into generally spherical shapes or irregular shapes. Also, sintered tungsten carbide in a crushed form is available. The hardness of standard spherical sintered tungsten carbide

pellets 39 ranges from about 1368 KHN (Knoop hardness), which is approximately 89.5 HRA (hardness Rockwell A), to about 1587 KHN (approximately 91.7 HRA).

Spherical cast tungsten carbide pellets 41 are formed in a casting process, and thus, are harder than sintered tungsten carbide and do not have a binder of a soft metal such as cobalt. Cast tungsten carbide particles may be spherical, irregular or crushed. Spherical cast tungsten carbide pellets 41 are typically smaller in diameter than standard spherical sintered tungsten carbide pellets 39. Hardness levels for spherical cast tungsten carbide pellets 41 range from about 1992 KHN (approximately 95.7 HRA) to about 2223 KHN (approximately 97.9 HRA). Typical sizes for spherical cast tungsten carbide pellets 41 in bit hardfacing are in the range from 44-250 microns. Spherical cast tungsten carbide pellets 41 are thus harder than standard spherical sintered tungsten carbide pellets 39 but more brittle. Standard spherical sintered tungsten carbide pellets 39 are tougher than spherical cast tungsten carbide pellets 41. Prior art hardfacing for earth-boring bits contains a variety of sizes and volume fractions of standard spherical sintered tungsten carbide pellets, crushed sintered tungsten carbide particles, spherical cast tungsten carbide pellets, crushed cast tungsten carbide particles, as well as other types of cast tungsten carbide, such as monocrystalline or macrocrystalline particles. The matrix that contains and binds the hardfacing pellets and particles is often iron, but it also may contain nickel or other alloys.

Referring to FIG. 3, in this embodiment, harder spherical sintered tungsten carbide pellets 43, referred to herein as "ultrahard pellets," are substituted for the spherical cast tungsten carbide pellets 41. Ultrahard pellets 43 differ in composition from standard spherical sintered tungsten carbide pellets 39 used in bit hardfacing. During the manufacturing of the powder used for ultrahard particles, submicron size tungsten carbide grains are blended with a binder of cobalt along with vanadium powder. During the sintering process, the vanadium inhibits the tungsten carbide grains from growing larger. Since the tungsten carbide grains remain small, the resulting sintered composition is very hard compared to standard sintered tungsten carbide. Iron and nickel might also be used as a binder either as a whole or in some combination with the cobalt binder. The vanadium thus serves as a tungsten carbide grain growth inhibitor. The quantity of vanadium may be as little as 0.25 percent and as much as 2 percent by weight of the total weight of the ultrahard pellet 43. A typical composition may be 4 percent to 8 percent cobalt, preferably 6 percent, 0.25 percent to 2 percent vanadium, and with the remainder being tungsten carbide. Ultrahard pellets 43 range in hardness from about 95 to 96 HRA. The sizes of ultrahard pellets 43 may be the same as standard spherical sintered tungsten carbide pellets 39, such as from 16 mesh to 325 mesh. For torch applications, such as on cones 19 (FIG. 1), the size range may be from about 177 to 250 microns, which is a typical prior art size range for spherical cast tungsten carbide pellets for torch applications. For pulse transferred arc (PTA) applications, such as on bit legs 17 (FIG. 1), the size range may be about 44 to 250 microns, which is approximately the size range used in the prior art for spherical cast tungsten carbide pellets with PTA applications. The sizes can be larger if ultrahard pellets are to be used to replace conventional spherical sintered tungsten carbide pellets used in torch applications, for example, up to about 1190 microns. Ultrahard pellets 43 may be spherical or irregular in shape, or sintered tungsten carbide having the same composition as ultrahard pellets 43 may be crushed.

## 5

In the example of FIG. 3, ultrahard pellets 43 are substituted for spherical cast tungsten carbide pellets 41. In this composition, ultrahard pellets 43 are mixed with standard spherical sintered tungsten carbide pellets 39 in the same percentage and roughly the same size ranges as the spherical cast tungsten carbide pellets 41 in FIG. 2.

In FIG. 4, ultrahard pellets 43 are mixed with spherical cast tungsten carbide pellets 41 and standard spherical sintered tungsten carbide pellets 39. The percentages may vary. The sizes of spherical cast tungsten carbide pellets 41 and ultrahard pellets 43 are relatively the same in this example, but they could vary also.

In FIG. 5, a crushed form of spherical ultrahard pellets 43 is used and referred to herein as "crushed ultrahard particles 45." Being crushed, ultrahard particles 45 are irregular in shape rather than spherical. Crushed ultrahard particles 45 may be roughly the same size range as spherical ultrahard pellets 43 or the sizes may differ. In the example of FIG. 5, crushed ultrahard particles 45 are mixed with spherical ultrahard pellets 43 and standard spherical sintered tungsten carbide pellets 39.

In FIG. 6, standard spherical sintered tungsten carbide pellets 39 and ultrahard pellets 43 are mixed with crushed cast tungsten carbide particles 47. Crushed cast particles 47 are irregular in shape and may be a variety of sizes. In the example shown, the sizes of crushed cast particles 47 are approximately the same as the sizes of ultrahard pellets 43.

In FIG. 7, standard spherical sintered tungsten carbide pellets 39 and spherical ultrahard pellets 43 are mixed with monocrystalline particles 49. Monocrystalline particles 49 comprise a single crystal of tungsten carbide and have an irregular shape. If larger than about 20 microns, they may be called macrocrystalline particles. During application, the sharp corners of the monocrystalline particles tend to melt, causing some of the tungsten carbide within to precipitate into the metal matrix. Monocrystalline particles 49 are conventional and available in a variety of sizes. In this example, they are approximately the same size as crushed ultrahard particles 43.

FIG. 8 discloses a combination of standard spherical sintered tungsten carbide pellets 39, spherical cast tungsten carbide pellets 41, spherical ultrahard pellets 43, crushed ultrahard particles 45 and monocrystalline particles 49. The percentages and sizes of each may be varied.

The examples of FIGS. 3-8 may be employed with any or all of the hardfacing layers 27, 29, 31 or 35 shown in FIG. 1. Further, the examples of FIGS. 3-8 may be used for hardfacing other downhole tools.

The various compositions described result in an extremely wear and/or erosion resistant material. The ultrahard particles provide more hardness than conventional sintered tungsten carbide particles. Although not as hard as cast tungsten carbide particles, ultrahard particles provide more toughness. Ultrahard particles may be used as a replacement for or in addition to cast tungsten carbide particles.

While several examples have been shown, it should be apparent to those skilled in the art that various changes may be made to these compositions.

What is claimed is:

1. A method of forming a hardfacing composition, comprising:

forming ultrahard pellets each comprising tungsten carbide grains, elemental cobalt, and elemental vanadium; crushing at least a portion of the ultrahard pellets to form crushed ultrahard particles;

mixing the crushed ultrahard particles with spherical sintered tungsten carbide pellets; and

## 6

dispersing the crushed ultrahard particles and the spherical sintered tungsten carbide pellets in a matrix metal comprising iron, nickel, or alloys thereof.

2. The method of claim 1, wherein forming ultrahard pellets comprises:

forming a powder mixture comprising tungsten carbide grains, a cobalt binder, and vanadium powder; and sintering the powder mixture.

3. The method of claim 1, wherein forming ultrahard pellets comprises forming each of the ultrahard pellets to comprise from 0.25 percent by weight to 2 percent by weight elemental vanadium.

4. The method of claim 3, wherein forming ultrahard pellets further comprises forming each of the ultrahard pellets to comprise from 4 percent by weight to 8 percent by weight of the elemental cobalt.

5. The method of claim 1, wherein forming ultrahard pellets comprises forming each of the ultrahard pellets to have a hardness within a range of from about 95 HRA to about 96 HRA.

6. The method of claim 1, wherein forming ultrahard pellets comprises forming at least one of the ultrahard pellets to have a spherical shape.

7. The method of claim 1, wherein:

crushing at least a portion of the ultrahard pellets to form crushed ultrahard particles comprises crushing only a portion of the ultrahard pellets to form the crushed ultrahard particles;

mixing the crushed ultrahard particles with spherical sintered tungsten carbide pellets comprises mixing the crushed ultrahard particles with the spherical sintered tungsten carbide pellets and a remaining portion of the ultrahard pellets; and

dispersing the crushed ultrahard particles and the spherical sintered tungsten carbide pellets in a matrix metal comprises dispersing the crushed ultrahard particles, the spherical sintered tungsten carbide pellets, and the remaining portion of the ultrahard pellets in the matrix metal.

8. A method of forming a hardfacing composition, comprising:

forming ultrahard pellets each comprising tungsten carbide grains, elemental cobalt, and elemental vanadium; crushing a portion of the ultrahard pellets to form crushed ultrahard particles;

mixing the ultrahard pellets and the crushed ultrahard particles with spherical sintered tungsten carbide pellets, spherical cast carbide pellets, and monocrystalline particles comprising tungsten carbide; and

dispersing the ultrahard pellets, the crushed ultrahard particles, the spherical sintered tungsten carbide pellets, the spherical cast carbide pellets, and the monocrystalline particles in a matrix metal comprising iron, nickel, or alloys thereof.

9. A method of hardfacing a downhole tool, comprising:

forming ultrahard pellets comprising tungsten carbide grains, elemental cobalt, and elemental vanadium; crushing a portion of the ultrahard pellets to form crushed ultrahard particles;

mixing the ultrahard pellets and the crushed ultrahard particles with spherical sintered tungsten carbide pellets;

dispersing the ultrahard pellets, the crushed ultrahard particles, and the spherical sintered tungsten carbide pellets in a matrix metal comprising iron, nickel, or alloys thereof to form a hardfacing composition; and

applying the hardfacing composition over at least one portion of the downhole tool to form a hardfacing layer over the downhole tool.

**10.** The method of claim **9**, wherein applying the hardfacing composition over at least one portion of the downhole tool comprises applying the hardfacing composition using a plasma transferred arc process.

**11.** The method of claim **9**, wherein applying the hardfacing composition over at least one portion of the downhole tool comprises applying the hardfacing composition using an oxyacetylene torch and a rod.

**12.** A method of forming an earth-boring bit, comprising: forming a bit body, bit legs, and cones rotatably mounted to the bit legs; and forming at least one hardfacing layer over outer surfaces of the bit legs, the at least one hardfacing layer comprising: ultrahard pellets comprising tungsten carbide, elemental vanadium, and at least one of cobalt, iron, and nickel; and

a matrix metal comprising iron, nickel, or alloys thereof, the ultrahard pellets dispersed in the matrix metal.

**13.** The method of claim **12**, further comprising forming the at least one hardfacing layer over one or more of teeth of the cones and gage surfaces of the cones.

**14.** A method of forming an earth-boring bit, comprising: forming a bit body, bit legs, and cones rotatably mounted to the bit legs; and forming at least one hardfacing layer over one or more of leading edges and trailing edges of the bit legs, the at least one hardfacing layer comprising: ultrahard pellets comprising tungsten carbide, elemental vanadium, and at least one of cobalt, iron, and nickel; and a matrix metal comprising iron, nickel, or alloys thereof, the ultrahard pellets dispersed in the matrix metal.

\* \* \* \* \*